

## UNITED STATES PATENT OFFICE.

MAURICE ERNEST BOUVIER, OF LYON, FRANCE, ASSIGNOR, BY MESNE ASSIGNMENTS,  
TO LA SOCIÉTÉ POUR LA FABRICATION DE LA SOIE "RHODIASETA," OF PARIS,  
FRANCE, A CORPORATION OF FRANCE.

## DYEING OF CELLULOSE ACETATE, ARTIFICIAL SILK, FILMS, AND THE LIKE.

No Drawing.

Application filed April 25, 1922. Serial No. 556,423.

*To all whom it may concern:*

Be it known that I, MAURICE ERNEST BOUVIER, residing at Lyon, France, a citizen of the Confederation of Switzerland, have **5** invented certain new and useful Improvements in or Relating to Dyeing of Cellulose Acetate, Artificial Silk, Films, and the like, of which the following is a specification.

This invention relates to the dyeing of **10** cellulose acetate films, threads or the like, and is an improvement in or a modification of the invention described in Letters Patent of the United States, No. 1,366,023, granted to Edmond Prince under date of January **15** 18, 1921.

In this patent, a process is described by **20** which cellulose acetate films, threads or the like are rendered capable of being dyed by being treated with solutions of salts of alkali metals to which alkali has been added.

In the said patent, only one example has been given, in which a solution of sodium chloride is used, to which caustic soda has been added. We have found that the caustic **25** alkali can be replaced by a salt with an alkaline reaction (carbonate, borate, silicate, tribasic phosphate, etc.) adapted to act as an alkali in the saponification of the acetate, the quantity of said salt being less than is **30** required to make a one per cent solution.

*Example.*

A hank of 100 grammes of cellulose acetate silk is plunged into a bath of 2 litres,

containing 800 gr. of crystallized sodium **35** sulphate (350 gr.  $\text{SO}_4\text{Na}_2$ ) and 17 gr. of sodium carbonate.

The hank is smoothed in the bath, gradually heated to  $85^{\circ}$  C. until paper impregnated with phenolphthalein is no longer colored by contact with it, this being obtained after a treatment of from 30 to 45 minutes.

The silk is then withdrawn from the bath and dyed.

What I claim and desire to secure by **45** Letters Patent is:—

1. A process for treating cellulose acetate films, silk and the like previous to dyeing, consisting in treating the cellulose acetate with a relatively concentrated solution of **50** neutral salts of alkali metals to which a salt with an alkaline reaction, adapted to act as an alkali in the saponification of the acetate is added in quantity less than is required to make a 1 per cent solution. **55**

2. The process of preparing cellulose acetate for dyeing, which consists in immersing the same in a bath containing sodium sulphate and sodium carbonate in the proportions of fifty to one, and heating the **60** bath to a temperature of approximately  $85^{\circ}$  C. for thirty to forty-five minutes.

In testimony whereof I have signed my name to this specification.

MAURICE ERNEST BOUVIER.

Witness:

JULIAN KEMBLE SNEDLEY.